

## 1

3,408,193

COATING COMPOSITIONS FOR THE COATING  
OUT OF ANIONIC MORDANT-ACID DYE  
LAYERS

Wilfred L. Wolf and Clark Beckett, Rochester, N.Y., as  
signors to Eastman Kodak Company, Rochester, N.Y.,  
a corporation of New Jersey  
No Drawing. Filed Dec. 16, 1964, Ser. No. 418,881  
8 Claims. (Cl. 96—84)

This invention relates to mordant-dye layers in which certain particular coating aids are employed in their composition.

Jones and Milton application Ser. No. 167,666, now Patent No. 3,282,699 describes mordant-dye compositions for use as layers in photographic elements such as for filter layers or antihalation layers which compositions are composed of a basic mordant having recurring basic groups, an acid dye, a water permeable hydrophilic colloid binder and as the coating aid therein saponin. Saponin varies widely in purity and often contains material which desensitizes or has other derogatory effects upon the silver halide emulsion with which it comes in contact. Therefore, it is desirable in photographic uses to use synthetic coating aids which have a uniform composition and are free of materials which might exert a derogatory effect on the photographic materials which they contact. In using the common coating aids such as of the anionic type in mordant-dye compositions high concentrations thereof are often needed to obtain satisfactory coatings. In addition these anionic coating aids tend to promote wandering of the dyes in the compositions into adjacent photographic emulsion layers resulting in desensitization of those layers.

The specification of application Ser. No. 167,666, filed Jan. 22, 1962, describes photographic elements containing layers composed of basic mordant, acid dye and hydrophilic colloid and is incorporated herein by reference.

One object of our invention is to provide mordant-acid dye coating compositions which use a synthetic coating aid in the coating out of those compositions onto a support. Another object of our invention is to provide basic mordant-acid dye compositions containing coating aids which do not promote the wandering of the dyes into adjacent silver halide photographic emulsion layers or require use in high proportions as is the case with many of the coating aids commonly considered useful in coating out photographic layers. Other objects of our invention will appear herein.

We have found that basic mordant-acid dye coating compositions which contain as the coating aids therein salts of alkyl substituted or acyl substituted amino acids as described in U.S. Patents Nos. 3,133,816 and 3,142,568 and in U.S. application Ser. No. 225,108 give coatings of good uniformity. The disclosures of the patents (Nos. 3,133,816 and 3,142,568) and the application (No. 225,108) referred to are incorporated herein by reference. We have found that concentrations in the coating compositions of no more than 5% of these coating aids based on the gelatin can be used with good results although greater amounts can be used if desired. We have found that coating aids of this type do not cause wandering of the dye into adjacent silver halide photographic emulsion layers, hence, desensitization of the emulsion layer is avoided. We have found that compositions in accordance with our invention are susceptible to coating out as layers at speeds of 50-500 feet per minute in coating operations in which hoppers of the type described in U.S. Patents Nos. 2,681,294 and 2,761,791 are used.

## 2

The following examples will illustrate our invention:

## Example 1

A gelatin, basic mordant-acid dye solution was prepared containing 454 parts of gelatin, 227 parts of the mordant polyalpha-methyl-allyl-N-guanidylketimine (glycolic acid salt), 75.6 parts of yellow sulfonated benzoxazole-pyrazolone dye and sufficient water to make a 1.4% gelatin solution. The coating aids listed below were added to separate portions of the solution which portions were then separately coated out over silver halide gelatin emulsion layer on a film support with the following results:

|    | Coating aid                                                    | Parts coating aid per 100 parts gelatin by wt. | Repellency coating defects |
|----|----------------------------------------------------------------|------------------------------------------------|----------------------------|
| 15 | Triton-X 200 (p-tert-octylphenoxy ethoxy ethyl sulfonate)----- | 7                                              | High.                      |
| 20 | Triton-X 200-----                                              | 10.6                                           | Fewer.                     |
| 20 | Deriphath 151 (sodium N-coco-beta-aminopropionate*)-----       | 2                                              | None.                      |

\*Where coco represents a mixture of high molecular weight hydrocarbon radicals corresponding to those present in the esters in cocoanut oil.

## Example 2

Two multilayer color films were prepared and coated as described in Example 16 of U.S. Patent No. 2,944,900 except that a yellow filter layer of the type described in Example 1 was used instead of the Carey Lea silver-blue light filter layer and a gelatin-basic mordant-magenta acid dye layer was coated between the green sensitive and red sensitive layers. In preparing one film an anionic coating aid was used in the mordant-dye layers and in the other a sodium salt of an alkyl aminopropionate as listed in Patent No. 3,133,816 was employed. The films were exposed on a sensitometer and were processed as described in Example 2 of U.S. Patent No. 2,944,900. The results obtained were as follows:

| 40 | Coating aid                                             | Parts coating aid per 100 parts gelatin by wt. |       |      | Relative speed |       |      |
|----|---------------------------------------------------------|------------------------------------------------|-------|------|----------------|-------|------|
|    |                                                         | Red                                            | Green | Blue | Red            | Green | Blue |
| 45 | Triton-X 200-----                                       | 11                                             | 8.8   | 7    | 83             | 83    | 80   |
| 45 | Deriphath 151 (sodium N-coco-beta-aminopropionate)----- | 1.8                                            | 2.8   | 2    | 100            | 100   | 100  |

The invention has been described in considerable detail with particular reference to certain preferred embodiments thereof, but it will be understood that variations and modifications can be effected within the spirit and scope of the invention as described hereinabove and as defined in the appended claims.

We claim:

1. A composition adapted to the coating out of layers for photographic products comprising in an aqueous system a hydrophilic colloid, a polymeric mordant having recurring basic groups, an acid dye and a coating aid selected from the group consisting of the compounds having the following general formulae:



and



wherein A is selected from the group of aliphatic hydrocarbon radicals and aliphatic acyl radicals of 8-20 carbon atoms,  $x=1-2$  and M is a cation which will contribute to the water solubility of the coating aid.

2. A photographic element having as a layer therein a mixture of a hydrophilic colloid, a polymeric mordant having recurring basic groups, an acid dye and a coating

aid selected from the group consisting of the compounds having the following general formulae:



and



wherein A is selected from the group of aliphatic hydrocarbon radicals and aliphatic acyl radicals of 8-20 carbon atoms,  $x=1-2$  and M is a cation which will contribute to the water solubility of the coating aid.

3. A composition adapted to the coating out of layers for photographic products comprising in an aqueous system a hydrophilic colloid, a polymeric mordant having recurring basic groups, an acid dye and as the coating aid therein a compound having the formula:



in which  $x=1-2$  and R is a radical having 11-17 carbon atoms and M is a cation contributing to water solubility of the coating aid.

4. A composition adapted to the coating out of layers for photographic products comprising in an aqueous system a hydrophilic colloid, a polymeric mordant having recurring basic groups, an acid dye and as the coating aid therein a compound having the formula:



wherein R is an aliphatic hydrocarbon radical having from 8 to 20 carbon atoms and X is selected from the group consisting of hydrogen, an alkali metal, ammonium and an organic amine cation.

5. A composition adapted to the coating out of layers for photographic products comprising in an aqueous system a hydrophilic colloid, a polymeric mordant having recurring basic groups, an acid dye and as the coating aid therein a compound having the formula:



wherein R is an aliphatic hydrocarbon radical having from 8 to 20 carbon atoms and X is selected from the group consisting of hydrogen, an alkali metal, ammonium and an organic amine cation.

6. A composition adapted to the coating out of layers for photographic products comprising in an aqueous system a hydrophilic colloid, a polymeric mordant having recurring basic groups, an acid dye and as the coating aid therein sodium N-coco-beta-aminopropionate.

7. A composition adapted to the coating out of layers for photographic products comprising in an aqueous system gelatin as the hydrophilic colloid, poly-alpha-methylallyl-N-guanidyl-ketimine as the mordant, yellow sulfonated benzoxazole-pyrazolone dye and as the coating aid a compound selected from the group consisting of those having the following general formulae:



and



wherein A is selected from the group of aliphatic hydrocarbon radicals and aliphatic acyl radicals of 8-20 carbon atoms,  $x=1-2$  and M is a cation which will contribute to the water solubility of the coating aid.

8. A composition adapted to the coating out of layers for photographic products comprising in an aqueous system gelatin as a hydrophilic colloid, poly-alpha-methylallyl-N-guanidylketimine as the mordant, yellow sulfonated benzoxazole-pyrazolone as the acid dye and as the coating aid sodium N-coco-beta-aminopropionate.

#### References Cited

##### UNITED STATES PATENTS

|    |           |         |              |           |
|----|-----------|---------|--------------|-----------|
| 30 | 2,240,471 | 4/1941  | Swan         | 96-109 XR |
|    | 2,882,156 | 4/1959  | Minsk        | 96-84     |
|    | 3,016,306 | 1/1962  | Mader et al. | 96-84 XR  |
|    | 3,133,816 | 5/1964  | Ben-Ezra     | 96-94     |
| 35 | 3,142,568 | 7/1964  | Nottorf      | 96-87     |
|    | 3,282,699 | 11/1966 | Jones et al. | 96-84     |
|    | 3,306,749 | 2/1967  | Knox et al.  | 96-94     |

NORMAN G. TORCHIN, Primary Examiner.

40 J. TRAVIS BROWN, Examiner.

R. H. SMITH, Assistant Examiner.